

R. L. SEABURY.

COMMUTATOR BRUSH AND METHOD OF MAKING THE SAME.

APPLICATION FILED JULY 27, 1914.

1,198,873.

Patented Sept. 19, 1916.

Fig. 2.



Fig. 1.



Fig. 3. B



Fig. 4.



WITNESSES:

H. Martin Canner  
A. D. Dempsey

INVENTOR

Ralph L. Seabury

# UNITED STATES PATENT OFFICE.

RALPH LOWE SEABURY, OF WELLSVILLE, NEW YORK.

## COMMUTATOR-BRUSH AND METHOD OF MAKING THE SAME.

1,198,873.

Specification of Letters Patent. Patented Sept. 19, 1916.

Application filed July 27, 1914. Serial No. 853,503.

To all whom it may concern:

Be it known that I, RALPH LOWE SEABURY, a citizen of the United States, residing at Wellsville, State of New York, have 5 invented certain new and useful Improvements in Commutator-Brushes and Methods of Making the Same, of which the following is a specification.

The object of my invention is the production of an improved brush for use on commutators and collector rings of dynamo electric machines which possesses good electrical characteristics and good wearing qualities and a good mechanical construction.

15 More particularly my invention relates to brushes that transmit heavy currents to or from the commutator and to brushes that are employed at low voltages and includes not only the article but the process of making it. Heretofore brushes for transmitting heavy currents and for use on low voltage machines have commonly been made of superimposed strips of thin copper or other metal or wire gauze (usually of bronze or of 25 copper) properly rolled and flattened into a nearly solid mass of the desired shape. Such brushes have not been satisfactory on account of excessive commutator and brush wear.

30 Another method commonly used to make brushes of high conductivity has been to employ very finely divided copper or other metal such as would pass through a one hundred (100) mesh screen intimately mixed 35 with finely divided carbon and the whole mass then being bonded together with pitch and subsequently baked or carbonized. This method is objectionable because too high a percentage of copper or metal is 40 necessary in order to secure a high conductivity thus reducing the percentage of carbon that can be used which results in a tendency of the brush to wear away itself and the commutator. Furthermore, such brushes sometimes fail to operate on low voltage work 45 owing to a thin film or coating presumably an oxid or carbid deposited on its face or on the commutator.

Still another method of making high con-

ductivity brushes has been to employ alternate layers of wire gauze, the strands which would measure about .010" in diameter and woven to about thirty (30) meshes per inch bonded between strips of carbon. Such brushes have a great tendency to break apart unless the layers of gauze are considerably separated and are open to the further objection that the strands of wire frequently fuse and melt away at the face of the brush when transmitting heavy currents caused by the current being carried by a comparatively few number of wires thus greatly impairing the conductivity of the brush.

Various other forms and combinations of brushes have been devised but none, so far as I am aware, has proved thoroughly efficient and satisfactory, for carrying very heavy currents or for operation on low voltage machines.

My invention aims to combine the high conductivity of metal with the lubricating qualities of carbon without encountering the difficulties and objections attending the older forms of brushes. In making my brush I employ copper or other metal in the form of narrow ribbons and exceedingly thin (about .001" in thickness) or preferably finely drawn wire about .003" in diameter, which preferably has been cut into short pieces about one eighth of an inch ( $\frac{1}{8}$ ") or if desired of about the same length as the thickness of the finished brush, then thoroughly mix these short metal filaments or ribbons with a certain percentage of finely ground carbon and add enough pitch or other binder to hold the mass firmly together after having been properly compressed and baked or otherwise cured. It may be remarked that the conductivity will be mainly governed by the percentage of metal filaments or ribbons present in the mix and that different commutating effects may be secured by not only changing the cross section of the metal filaments or ribbons themselves, either above or below the dimensions given above but also by changing their lengths as used in the mix.

In the preferred form of my invention I employ a mixture containing about sixty

per cent. of copper filaments, about twenty-five per cent. of carbon and about fifteen per cent. of pitch. Any suitable method may be employed in forming or compressing the mix into suitable form. The method which I ordinarily employ consists of molding the mix in suitable molds under a pressure of about thirteen tons per square inch.

Another method which can be employed 10 is that which is called extruding or squirt- ing in which the mix is forced through a suitable aperture of a hydraulic press com- monly called "jumbo." The brushes are then baked to a temperature of about 840 15 degrees C. which temperature is sufficient to carbonize the binder and render the brush solid and hard. During the process of mold- ing or extruding such brushes on account of the particular forms that I have de- 20 scribed of comparatively short ribbons or filaments in the mix, practically all the fila- ments or ribbons will arrange themselves so that their major axis will lie parallel to the sides of the brush. I attribute the forma- 25 tion of this arrangement to the fact that considerable air is expelled from the mix during the process of molding which rap- idly escapes laterally and finally leaving be- 30 tween the walls of the mold and the plunger, the said air in thus escaping forces the fila- ments to a great extent to arrangethemselves in a plane parallel to the face of the plun- ger. During the extrusion process in a so- 35 called jumbo such filaments or ribbons being much longer than they are wide or thick, would on account of the dragging effect of the die, tend to force such elongated metal- lic particles to arrange themselves so that their length would lie in a plane parallel 40 with the plane of the thickness of the brush, thus producing substantially the same ef- fect as in molding the brush. This is a very desirable arrangement since practically each filament at the face of the brush will pre- 45 sent against the commutator one of its ends; this construction secures a very low contact resistance between the commutator and the brush. Furthermore, since each filament is in excellent electrical contact with the ones 50 adjacent to it, either by actual metallic con- tact or through a very thin medium of car- bon, brushes of this construction have an ex- ceedingly low specific resistance, one con- taining sixty per cent. filaments showing as 55 low a resistance as brushes commonly made that contain eighty per cent. metal in the usual powdered form. This not only ef- fects a saving in metal, important particu- larly if silver, gold or other expensive metal 60 is used, but also permits a much larger per- centage of carbon to be used in the brush, the chief object of which is to act as a lubri- cant and to prevent abrasion or undue wear-

ing and scoring of the brush and commuta- tor. And furthermore, brushes made in 65 this manner are much stronger and tougher and even slightly flexible when in a thin sec- tion than brushes ordinarily made by the use of powdered copper or wire gauze, due to their fibrous composition and structure. 70

Another construction which can be em- ployed consists in making the brush in a composite form, the outside sections being made of carbon while the central core or strip is made of a mixture of metallic fila- 75 ments and carbon such as I have previously described.

Numerous other modifications and combi- nations from the above description would of course be obvious to those skilled in the art. 80

In the accompanying drawings Figure 1, is an elevation showing the completed brush; Fig. 2, is an end view showing the ends of the metal filament in the face of the brush; Fig. 3, illustrates an end view of a com- 85 posite brush while Fig. 4, shows a diagram- matic side view of a composite brush.

Referring to the drawing, A designates a brush in which the metallic particles 1 are distributed throughout the body of the brush, 90 being embedded in the material 2 formed by the carbon and pitch, as shown in Fig. 1. The metallic particles 1 extend longitudinally of the brush, and in Fig. 2 only the ends of the particles lying in the end sur- 95 face of the brush are seen. In Figs. 3 and 4 a brush B is shown in which the core is composed of metal particles embedded in carbon and pitch, and around the core is a covering 3 of carbon and pitch material. 100

The above described arrangements are deemed sufficient to illustrate the nature of my invention and are intended as enumera- tions of all of its modifications.

This brush may be used in other situations 105 where it is desired to change or switch heavy currents or where a contact for low voltage work is desired that will minimize the volt- age drop. This also may be used as a self lubricating bearing material. 110

While I have hereinbefore described and illustrated the best form of my invention now known to me, it is obvious that those skilled in the art may make changes and modifications in the form of my invention 115 without departing from its spirit.

What I claim as new and desire to secure by Letters Patent of the United States, is:

1. A commutator brush comprising a 120 block of carbon, having embedded therein a quantity of fine metallic strands, said strands being promiscuously disposed throughout the block and the strands being substan- tially parallel with the major axis of the brush.

2. The herein-described process of mak-

ing electric brushes, which consists in mixing carbon particles, a suitable binder, and metallic particles of elongated form into a plastic mass, with the metal particles 5 miscuously arranged; extruding the mass under pressure through a form simultaneously to shape the brush and cause the metal particles to become parallelized with respect

to themselves and to the axis of the brush, and baking the brush.

July 24, 1914.

RALPH LOWE SEABURY.

Witnesses:

L. H. DAVIS,  
W. J. RICHARDSON.